

United States Patent [19]  
Noë

[11] 3,865,587  
[45] Feb. 11, 1975

[54] ELECTROPHOTOGRAPHIC BICHARGEABLE MATERIALS AND PROCESS

[75] Inventor: Robert Joseph Noë, Mortsel, Belgium

[73] Assignee: Agfa-Gevaert N.V., Mortsel, Belgium

[22] Filed: July 19, 1972

[21] Appl. No.: 273,056

[30] Foreign Application Priority Data

July 20, 1971 Great Britain 34046/71

[52] U.S. Cl. 96/1 PC, 96/1.7, 96/1.8

[51] Int. Cl. G03g 5/08, G03g 13/22

[58] Field of Search 96/1.8, 1 PC; 252/501

[56] References Cited

UNITED STATES PATENTS

|           |         |                 |          |
|-----------|---------|-----------------|----------|
| 2,287,161 | 6/1942  | Ball            | 96/1.8 X |
| 2,555,321 | 6/1951  | Dalton et al.   | 96/1.8 X |
| 2,952,536 | 9/1960  | Kurz            | 96/1.8 X |
| 2,983,220 | 5/1961  | Dalton et al.   | 96/1.8 X |
| 3,060,134 | 10/1962 | Elder et al.    | 96/1.8 X |
| 3,174,856 | 3/1965  | Horne et al.    | 96/1.8 X |
| 3,607,255 | 9/1971  | Back            | 96/1.8 X |
| 3,634,135 | 1/1972  | Akiyama         | 96/1.8 X |
| 3,642,480 | 2/1972  | Vrancken        | 96/1.8 X |
| 3,652,271 | 3/1972  | Barmarth et al. | 96/1.8   |
| 3,653,895 | 4/1972  | Brandon         | 96/1.8 X |
| 3,674,477 | 7/1972  | Carlson         | 96/1.8   |
| 3,674,483 | 7/1972  | Vrancken et al. | 96/1.8 X |

|           |         |         |          |
|-----------|---------|---------|----------|
| 3,703,371 | 11/1972 | Merrill | 96/1.8 X |
| 3,703,372 | 11/1972 | Merrill | 96/1.8 X |
| 3,706,560 | 12/1972 | Grain   | 96/1.8 X |
| 3,801,316 | 4/1974  | Bowman  | 96/1.8 X |

FOREIGN PATENTS OR APPLICATIONS

|         |         |               |        |
|---------|---------|---------------|--------|
| 908,779 | 10/1962 | Great Britain | 96/1.8 |
| 941,702 | 11/1963 | Great Britain | 96/1.8 |

OTHER PUBLICATIONS

Hauffe et al., "Electrophotographic Charging and Discharging Experiments with Zinc Oxide Single Crystals," *Phys. Stat. Sal.* (a) 3, No. 1, pp. 173-183 (1970).

Hoeffgen et al., "On the Electrophotographic Behaviour of Pink Zinc Oxide," *Phys. Stat. Sal.* (a) 3, No. 1, pp. 185-192, (1970).

Primary Examiner—Norman G. Torchin

Assistant Examiner—John R. Miller

Attorney, Agent, or Firm—William J. Daniel

[57] ABSTRACT

An electrophotographic recording material comprising a photoconductive binder type layer incorporating a mixture of photoconductive zinc oxide particles and colourless or white positively chargeable pigment particles in a ratio by weight smaller than 50:50 but not smaller than 10:90.

Preferred positively chargeable pigment particles are zinc sulphide, barium sulphate, silica or polyethylene particles.

2 Claims, No Drawings

## ELECTROPHOTOGRAPHIC BICHARGEABLE MATERIALS AND PROCESS

This invention relates to an electrophotographic recording material and its use in the production of photographic images.

Photoconductive binder type coatings prepared by incorporating a finely divided photoconductor in a binder are well known.

Commonly used are electrophotographic materials containing a photoconductive layer comprising photoconductive zinc oxide dispersed in an insulating binder. Said layer is coated on a sufficiently conductive support, e.g. a clay-coated or glassine type paper base, from a paint-like coating mixture by conventional paper coating techniques.

Since the zinc oxide has a brilliant white colour it forms an excellent base for contrasting with the developer materials applied to it. Moreover, zinc oxide is relatively less expensive and can be spectrally sensitized by a great variety of dyes. However, as already explained in the United Kingdom patent specification No. 1,256,888 filed June 6, 1968 by Gevaert-Agfa N.V. the positive corona charging of photoconductive zinc oxide binder layers is only of an acceptable level if photoconductive zinc oxide is used that has been treated with a special chemical compound improving its positive chargeability.

The present invention is based on the discovery that electrophotographic recording materials containing photoconductive zinc oxide can be used for electrophotographic recording purposes including a positive charging by the use in the photoconductive binder type layer of a mixture of photoconductive particles and colourless or white positively chargeable pigment particles in a ratio by weight range being smaller than 50:50 but not smaller than 10:90.

Preferred mixtures of dispersed photoconductive zinc oxide and positively chargeable particles are in a ratio by weight range from 30:70 to 40:60.

Remarkable is that the positively chargeable particles need not to be photoconductive and that inorganic as well as organic finely divided positively chargeable particles may be used.

For selecting the positively chargeable particles a test has been developed according to the particles involved are dispersed in a ratio of 50 to 95% by weight in an insulating binder having a resistivity of at least  $10^{12}$  ohm.cm and coated on a conductive base forming a layer of 10-30 microns.

The coated layer is subjected in the dark to a positive corona charging of + 6000 V till a maximum voltage level is reached.

Thus prepared and treated layers that after terminating the charging step retain for at least 5 seconds in the dark a positive charge with a potential difference of at least 200 V with respect to a contacting conductive carrier or support contain pigments suited for the purpose of the present invention.

The dark decay is registered e.g. by means of an electrometer with vibrating electrode such as that described by C. J. Young and H. G. Greig, RCA Review (1954) XV, 469, switched to a Brüel & Kjaer Voltage Level Recorder.

Substances that are within the criteria of the above test and that for the purpose of the present invention

are used advantageously in combination with photoconductive zinc oxide are e.g. the following:

barium sulphate  
zinc sulphide  
silica ( $\text{SiO}_2$ )  
polyethylene

The grain size of the added substances is advantageously about the grain size of the photoconductive zinc oxide particles but may vary within a broad range 10 e.g. from  $10^{-2}$  micron to 20-50 micron.

The grain size of the photoconductive zinc oxide is, e.g. of 0.1 to 15 micron.

In admixture with a suitable insulating binder or binder mixture the recording layer has preferably a resistivity which is approximately between  $10^7$  and  $10^{14}$  ohm.cm.

The recording layer may contain from 50 to 97% by weight of the dispersed particles with respect to the binder material. A preferred ratio by weight of binder to dispersed particles is in the range of 1:4 to 1:10 parts.

Any polymeric or resinous binding agent or mixture of polymeric binding agents already known for use in electrophotographic recording layers containing photoconductive zinc oxide may be used.

Suitable binding agents have a resistivity that is higher than the inherent resistivity of the photoconductive zinc oxide particles. In that respect are used e.g. electrically insulating organic resinous binders of the type of polyurethanes, polyesters, polycarbonates, polystyrene, chlorinated rubber, acrylic resin, alkyd resins or vinyl acetate copolymers e.g. vinyl chloride-acetate resin.

According to the coating composition the binder/pigment layers are coated from an organic solvent or solvent mixture, an emulsion of organic solvents and water or from an aqueous medium.

Particularly suitable binding agent combinations for application from organic solvents are described in the United Kingdom patent specification No. 1,199,061 filed Apr. 26, 1967 by Gevaert-Agfa N.V.

Photoconductive coating compositions applied from an aqueous emulsion are described, e.g., in the U.S. Pat. No. 3,152,895 of Georges H. Tinker, Shu Huai, David Mai and Roger E. Burke issued Oct. 13, 1964.

Photoconductive coating compositions applied from an alkaline aqueous binder solution are described, e.g. in the United Kingdom patent specification Nos. 1,125,579 and 1,125,580 both filed Oct. 25, 1966 by Gevaert-Agfa N.V. and the U.S. Pat. No. 3,160,503 of Joseph H. Cady issued Dec. 8, 1964.

According to a special embodiment the binding agent or binding agent composition has a resistivity that is lower than that of photoconductive zinc oxide grains treated with a compound as described in United Kingdom patent specification Nos. 1,020,504 and 1,020,506 both filed Dec. 29, 1961 by Gevaert Photo-Producten N.V.

According to the inventions described in said Patent Specifications it has been found that a sufficient dark-resistivity can be conferred on the zinc oxide to make it unnecessary when forming a photoconductive zinc oxide layer to use a binder with a high dark-resistivity. Preferred compounds for treating the photoconductive zinc oxide grains and increasing its dark-resistivity are acid ester derivatives of oxyacids of phosphorus e.g. mono- and dibutyl orthophosphate.

60  
65

Other compounds improving the dark-resistivity of photoconductive zinc oxide grains are urazole, urazole derivatives and analogous compounds described in the United Kingdom patent specification No. 1,256,888 filed June 6, 1968 by Gevaert-Agfa N.V. and the U.S. Pat. No. 3,634,080 of Robert Joseph Noë, Jozef Frans Willems, Albert Lucien Poot and Karel Eugène Verhille issued Jan. 11, 1972. These compounds correspond with the following general formula:



wherein:

each of  $R_1$  and  $R_2$  represents hydrogen, an alkyl group including a substituted alkyl group, and aryl group including a substituted aryl group, an acyl group including a substituted acyl group, e.g. an aliphatic acyl group (alcoyl) or substituted aliphatic acyl group, e.g. an acetyl group, or an aromatic acyl group (aroyl), e.g. a benzoyl group, including a substituted aromatic acyl group, or a heterocyclic nucleus including a substituted heterocyclic nucleus, e.g. a pyridine nucleus, or a thiazole nucleus, or  $R_1$  and  $R_2$  together represent the necessary atoms to close a fused ring or ring system,  $Z$  the atoms necessary to close a 5- or 6-membered heterocyclic ring including such ring in substituted form and including such ring making part of an either or not substituted fused ring system, and  $X$  represents oxygen or imino, and at least one of the nitrogen atoms making part of the ring closed by  $Z$  carries a hydrogen atom, that optionally may be replaced by a cation when using the compound in salt form

Said compounds increasing the dark-resistivity are used in combination with the photoconductive zinc oxide in preferred amounts of 0.01 to 10% by weight.

In the manufacture of the electrophotographic material according to the present invention in practice any commercially available white zinc oxide prepared e.g. by oxidation of zinc vapour (French process) may be used.

Especially suited zinc oxide types are:

the zinc oxide marketed under the trade name BLANC DE ZINC Neige extra pure, type A, B and C, by Vieille Montagne S.A. Liege, Belgium, and the

zinc oxide marketed by Durham Chemical Ltd. Birtley England under the trade names MICROX and ELECTROX.

In addition to the binding agent(s) the positive chargeable particles, the photoconductive zinc oxide grains and the compounds increasing the dark-resistivity the recording layers of the present invention may contain all other additives known in the art, e.g., compounds influencing the mechanical strength, gloss, viscosity, thermal stability and compounds that increase the spectral sensitivity and/or general sensitivity of the recording layer.

Examples of suitable spectral sensitizing agents that increase the spectral sensitivity of photoconductive zinc oxide are described in the United Kingdom patent specification Nos. 1,020,504 filed Dec. 29, 1961 by

Gevaert Photo-Producten N.V. — 1,199,062 — 1,200,901 both filed Apr. 26, 1967, 1,183,044 filed Apr. 5, 1966 and 1,198,994 filed Dec. 20, 1966 all by Gevaert-Agfa N.V.

5 For masking the colour of the applied spectral sensitizing agent, dyes complementary in colour to the sensitizing agent giving the recording layer an off-white appearance may be applied as described, e.g. in the United Kingdom patent specification No. 1,142,509 10 filed May 20, 1966 by Gevaert-Agfa N.V.

According to a preferred embodiment for preparing photoconductive recording materials of the invention both the photoconductive zinc oxide particles and the positively chargeable particles are dispersed homogeneously in a solution containing the dissolved insulating binding agent(s) and the obtained dispersion is applied to an electro-conductive support.

15 In the coating of the photoconductive layer several techniques may be used, e.g. centrifuging, spraying, brushing, roller coating, dip-coating, knife-coating or extrusion.

The formed layer is dried, e.g., by a hot air current or by infrared radiation.

20 The support for the recording layer preferably has a resistivity that is 100 times as small as that of the dried recording layer in the dark. In general its resistivity is smaller than  $10^9$  ohm.cm, but preferably smaller than  $10^5$  ohm.cm.

25 The supports may be made of metal, resin sheets coated with conductive layers or paper supports that contain conductive substances and/or are coated with conductive interlayers. Particularly suitable paper supports are those that have a high impermeability to organic solvents such as glassine paper described in the United Kingdom patent specification No. 995,491 filed Mar. 16, 1962 by Gevaert Photo-Producten N.V.

30 Paper sheets that have an insufficient electric conductivity are coated or impregnated with substances enhancing their conductivity, e.g. by means of a conductive polymer overcoat or by means of a metal sheet e.g. aluminium sheet laminated to the paper.

35 Substances suited for enhancing the conductivity of a paper sheet and which can be applied in the paper mass are hygroscopic compounds and antistatic agents are described, e.g. in the United Kingdom patent specification No. 964,877 filed May 2, 1960 by Gevaert Photo-Producten N.V. and antistatic agents of the polyionic type, e.g. CALGON CONDUCTIVE POLYMER 40 261 (registered trade-mark of Calgon Corporation, Inc., Pittsburgh, Pa., U.S.A.) for a solution containing 39.1% by weight of active conductive solids, and which contain a conductive polymer having recurring units of the following type:



50 65 60 55 50 45 40 35 30 25 20 15 10 5 50 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155

Recording materials according to the present invention can be used in a recording technique comprising a negative corona charging as well as in a recording technique comprising a positive corona charging.

Thanks to this property it is possible, with one and the same developer, e.g. and electrophoretic developer with toner particles carrying, e.g., a positive charge, to reproduce one and the same original at will as a positive or a negative copy depending on the sign of the electrostatic charge applied to the recording layer of said recording material.

Thus, it is possible, e.g. by starting from a microfilm image as an original, to prepare positive as well as negative enlarge copies of that original by means of the recording materials of the present invention.

The following examples illustrate the present invention.

#### EXAMPLE 1

The improved positive chargeability and recording properties of photoconductive recording materials containing zinc sulphide in the range suited for the purpose of the invention is proved by the following series of comparative tests.

For comparison's sake the following coating compositions in which the ratio of photoconductive zinc oxide with respect to zinc sulphide was step-wise varied in 10 % by weight decrements were prepared.

Except for the photoconductive zinc oxide and zinc sulphide the ingredients of the coating compositions were the following for 1 l of solvent mixture:

a) binder composition : ALKYDAL V 15 (trade name for a styrolated alkyd resin of Bayer AG - W.-Germany) 75 % by weight solution in toluene 16 g

b) copolymer of ethylene, vinyl-sulphonyl chloride and vinyl chloride (26.1/6.9/67 % by weight) 80 g

urazole 0.32 g

spectral sensitizing agents : bromophenol blue 28 mg

and



silicone oil 0.2 ml

solvent mixture : dichloroethane 500 ml

ethanol 30 ml

toluene 300 ml

methyl ethyl ketone 170 ml

The average grain size of the photoconductive zinc oxide and the zinc sulphide were 0.17 micron and 1.8 micron respectively.

The obtained dispersion was dip-coated onto a glassine type paper support having a resistivity of 5.10<sup>8</sup> ohm.cm at 50 % relative humidity and a weight of 70 g per sq.m and dried in a laminar air current drier by conveying air at 40°C over the coating at a speed of 2 m per sec. The coated layer contained 35 g of pigment per sq.m.

Column A of the following Table 1 contains the amount of zinc oxide of each coating composition expressed in % by weight with respect to the total weight of zinc oxide and zinc sulphide.

Column B contains analogously to column A the % by weight of zinc sulphide.

In column C the maximum positive charge expressed by the obtained voltage level (V) built up under the same positive charge conditions is listed.

Column D the maximum negative charge expressed by the obtained voltage level (V) built up under the same negative charge conditions is listed.

In columns E and F is listed the percentage inherent decay of charge in the dark 3 sec after the end of the positive and negative charging respectively.

In columns G and H the percentage decay of charge under same light (incandescent lamp light) exposure conditions (750 lux.sec) is listed for the positively and negatively charged recording layers respectively. The charge decay under exposure is measured after a constant charge decay in the dark has been reached.

The total pigment content (ZnO + ZnS) was 400 g.

The ingredients were mixed in a ball-mill.

In column I the relative speed (expressed in steps) of the described materials obtained by a negative corona charging, exposure through a step-wedge of constant 0.1 and development with positive electrophoretic toner is listed.

In columns J and K are listed the contrast and image acutance appreciation of the obtained results on development of the produced positive charge images. For obtaining these results after the positive charging under the same conditions, the recording materials were exposed through a step wedge with constant 0.3 superposed on a transparency representing a copy of a printed text. Then the acutance of the produced letters in the areas of different contrast was examined.

## EXAMPLE 2

Example 1 was repeated with the difference, however, that the zinc sulphide was replaced by barium sulphate (average grain size : 1.7 micron)

The obtained results are listed and discussed in Table 2 hereinafter analogously to those in Table 1.

## EXAMPLE 3

Example 1 was repeated with the difference, however, that the zinc sulphide was replaced by silica (average grain size : 5 micron).

The obtained results are listed and discussed in Table 3 hereinafter analogously to those in Table 1.

Table 1

| A<br>(ZnO) | B<br>(ZnS) | C<br>(Volts+) | D<br>(Volts-) | E<br>(% Decay<br>in Dark) | F<br>(% Decay<br>in Dark) | G<br>(% Decay<br>in Dark) | H<br>(% Decay<br>in Dark) | I<br>(steps) | J<br>(contrast) | K<br>(acutance) |
|------------|------------|---------------|---------------|---------------------------|---------------------------|---------------------------|---------------------------|--------------|-----------------|-----------------|
| 100        | 0          | 210           | 800           | 86                        | 4                         | —                         | 87                        | 11           | no image        | —               |
| 90         | 10         | 160           | 840           | 90                        | 2                         | —                         | 76                        | 13           | very weak       | bad             |
| 80         | 20         | 190           | 830           | 92                        | 7                         | —                         | 72                        | 11           | weak            | bad             |
| 70         | 30         | 170           | 840           | 94                        | 9                         | —                         | 31                        | 14           | weak            | bad             |
| 60         | 40         | 190           | 830           | 90                        | 4                         | —                         | 20                        | 11           | weak            | bad             |
| 50         | 50         | 360           | 840           | 89                        | 2                         | —                         | 14                        | 11           | good            | bad             |
| 40         | 60         | 700           | 900           | 21                        | 2                         | 59                        | 11                        | 10           | good            | fairly good     |
| 30         | 70         | 1000          | 840           | 8.2                       | 2.5                       | 11                        | 13                        | 10           | good            | good            |
| 20         | 80         | 1030          | 840           | 6                         | 2.4                       | 6                         | 8                         | 5            | fairly good     | good            |
| 10         | 90         | 1040          | 840           | 5                         | 2.1                       | 5                         | 6                         | 1            | fairly weak     | good            |
| 0          | 100        | 1010          | 840           | 6                         | 4                         | 2                         | 2                         | none         | no image        | —               |

Table 2

| A<br>(ZnO) | B<br>(BaSO <sub>4</sub> ) | C   | D   | E  | F  | G  | H  | I<br>(steps) | J<br>(contrast) | K<br>(acutance) |
|------------|---------------------------|-----|-----|----|----|----|----|--------------|-----------------|-----------------|
| 100        | —                         | 210 | 800 | 86 | 4  | —  | 87 | 11           | no image        | —               |
| 90         | 10                        | 760 | 850 | 22 | 7  | 94 | 68 | 16           | weak            | bad             |
| 80         | 20                        | 820 | 840 | 18 | 9  | 92 | 42 | 14           | weak            | bad             |
| 70         | 30                        | 800 | 840 | 19 | 12 | 35 | 23 | 14           | weak            | fairly good     |
| 60         | 40                        | 810 | 840 | 18 | 14 | 66 | 43 | 16           | fairly good     | good            |
| 50         | 50                        | 840 | 840 | 17 | 16 | 41 | 35 | 15           | good            | good            |
| 40         | 60                        | 800 | 850 | 22 | 14 | 33 | 31 | 14           | good            | good            |
| 30         | 70                        | 760 | 860 | 21 | 17 | 27 | 26 | 11           | good            | good            |
| 20         | 80                        | 700 | 840 | 25 | 22 | 19 | 18 | 6            | weak            | good            |
| 10         | 90                        | 700 | 840 | 24 | 24 | 10 | 10 | 1            | weak            | good            |
| 0          | 100                       | 660 | 800 | 33 | 29 | 7  | 7  | none         | no image        | no image        |

Table 3

| A<br>(ZnO) | B<br>(SiO <sub>2</sub> ) | C    | D   | E  | F  | G  | H  | I<br>(steps) | J<br>(contrast) | K<br>(acutance) |
|------------|--------------------------|------|-----|----|----|----|----|--------------|-----------------|-----------------|
| 100        | —                        | 210  | 800 | 86 | 4  | —  | 87 | 11           | no image        | no image        |
| 90         | 10                       | 340  | 830 | 78 | 5  | —  | 90 | 13           | rather weak     | bad             |
| 80         | 20                       | 750  | 840 | 27 | 8  | 97 | 90 | 14           | rather weak     | bad             |
| 70         | 30                       | 790  | 840 | 27 | 8  | 97 | 75 | 14           | weak            | bad             |
| 60         | 40                       | 850  | 850 | 18 | 9  | 96 | 77 | 15           | weak            | bad             |
| 50         | 50                       | 900  | 840 | 12 | 11 | 63 | 95 | 14           | good            | bad             |
| 40         | 60                       | 970  | 850 | 12 | 11 | 53 | 95 | 14           | good            | good            |
| 30         | 70                       | 1020 | 830 | 10 | 16 | 25 | 40 | 14           | good            | good            |
| 20         | 80                       | 950  | 840 | 13 | 19 | 21 | 29 | 6            | fairly good     | good            |
| 10         | 90                       | 1030 | 850 | 10 | 13 | 17 | 19 | 1            | weak            | good            |
| —          | 100                      | 1150 | 960 | 4  | 5  | 4  | 2  | none         | no image        | no image        |

## EXAMPLE 4

Example 1 was repeated with the difference, however, that the zinc sulphide was replaced by polyethylene particles having an average grain size of 15 micron.

The obtained results analogously to those discussed in Table 1 for columns I, J and K are listed in Table 4 hereinafter.

Table 4

| A<br>(ZnO) | B<br>(polyethy-<br>lene) | I<br>(steps) | J<br>(contrast) | K<br>(acutance) |
|------------|--------------------------|--------------|-----------------|-----------------|
| 100        | 0                        | 14           | no image        | no image        |
| 90         | 10                       | 13           | weak            | bad             |
| 80         | 20                       | 16           | weak            | bad             |
| 70         | 30                       | 14           | rather weak     | bad             |
| 60         | 40                       | 19           | good            | bad             |
| 50         | 50                       | 17           | good            | good            |
| 40         | 60                       | 15           | good            | good            |
| 30         | 70                       | 7            | good            | good            |
| 20         | 80                       | 1            | fairly good     | good            |
| 10         | 90                       | 1            | fairly good     | good            |
| 0          | 0                        | none         | no image        | no image        |

## EXAMPLE 5

A homogeneous mixture containing the following ingredients was prepared in a sand mill:

|                                                                                                                                                                  |          |
|------------------------------------------------------------------------------------------------------------------------------------------------------------------|----------|
| dichloroethane                                                                                                                                                   | 7.4 l    |
| ethanol                                                                                                                                                          | 0.4 l    |
| cyclohexanone                                                                                                                                                    | 1 l      |
| 50 % by weight solution in toluene<br>of the terpolymer of vinyl acetate,<br>styrene, aliphatic acrylic acid<br>ester and acrylic acid (25/30/44/1<br>by weight) | 1.2 l    |
| ALKYDAL V 15 (trade name) as a 75 %<br>by weight solution in toluene                                                                                             | 240 ml   |
| zinc oxide, type ELECTROX (trade name)                                                                                                                           | 1,440 kg |
| colloidal silica (average particle<br>size 5 $\mu$ )                                                                                                             | 2,160 kg |
| 10 % by weight solution of urazole<br>in dimethylformamide                                                                                                       | 36 ml    |
| 1 % by weight solution of bromophenol<br>blue in methanol                                                                                                        | 19 ml    |
| 0.5 % by weight solution in dimethyl-<br>formamide of the cyanine sensitizing<br>dye of Example 1                                                                | 22 ml    |

The dispersion was roller-coated in a ratio of 40 g of solids per sq.m. The coated layer was dried in a laminar air current drier. As supported for the coated layer a glassine type paper of 72 g per sq.m being made more conductive with sodium sulphate and calcium chloride was used.

After charging with a positive corona the recording layer was exposed through a negative transparency of a printed text and developed in an electrophoretic developer having the following composition:

500 g of ALKYDAL L 67 (trade-name of Farbenfabriken Bayer AG, Leverkusen, W.-Germany, for a linseed oil (67 % by weight) modified alkyd resin) and 500 ccs of white spirit containing 11 % by weight of aromatic compounds are heated at 60°C till a clear solution A is obtained. After cooling the solution A to room temperature, 150 g thereof are used as fixing agent for the following dispersion.

|                                                                                                                                                                                                                                  |         |
|----------------------------------------------------------------------------------------------------------------------------------------------------------------------------------------------------------------------------------|---------|
| carbon black (average particle<br>size 20 m $\mu$ )                                                                                                                                                                              | 30 g    |
| zinc monotridecyl phosphate                                                                                                                                                                                                      | 1.5 g   |
| SHELLSOL T (trade name for a mixture<br>of aliphatic hydrocarbons having the<br>following characteristics:<br>density at 15°C: 0.764<br>boiling range: 180-200°C<br>viscosity at 25°C: 1.62 cP<br>Kauri-Butanol number (KB): 31) | 750 ccs |

Mixing of the solution A with the said composition occurs as follows:

150 g of said solution are first ground in a ball-mill with 1.5 g of the zinc monotridecyl phosphate, whereupon 30 g of carbon black are added and at least 750 ccs of Shellsol T (trade name).

15 After grinding the whole composition for 15 h the obtained concentrated developer is diluted with Shellsol T (trade name) in a ratio of 15/1000.

20 The developer thus obtained is very stable and yields quite erasure-proof images after evaporation of the solvent from the recording layer.

25 A contrasty image having reversed image values with respect to the original and with excellent actuation was obtained.

## EXAMPLE 6

A homogeneous mixture of the following ingredients 30 was prepared in a sand mill:

|                                                                                                                                                                                                                                                                  |          |
|------------------------------------------------------------------------------------------------------------------------------------------------------------------------------------------------------------------------------------------------------------------|----------|
| dichloroethane                                                                                                                                                                                                                                                   | 2,300 l  |
| ethanol                                                                                                                                                                                                                                                          | 0.300 l  |
| toluene                                                                                                                                                                                                                                                          | 2,300 l  |
| 35 n-butanol                                                                                                                                                                                                                                                     | 1,700 l  |
| ALKYDAL V 15 (trade name) as a 75 %<br>by weight solution in toluene                                                                                                                                                                                             | 210 ml   |
| ZnO - type MICROX (trade name)                                                                                                                                                                                                                                   | 1,600 kg |
| 40 silica (average grain size 5 $\mu$ )                                                                                                                                                                                                                          | 2,400 kg |
| HYPALON 30 (trade name for a copoly<br>(ethylene/vinylsulphonyl chloride/vinyl<br>chloride) (26.1/6.9/67 in % by weight)<br>marketed by E. I. du Pont de Nemours<br>& Co (Ind.) Wilmington, Del., U.S.A.) as<br>a 25 % by weight solution in dichloro-<br>ethane | 4,600 kg |
| a 3 % by weight solution of silicone<br>oil in dichloroethane                                                                                                                                                                                                    | 66 ml    |

50 The obtained dispersion was coated and processed as described in Example 5.

A contrasty image having reversed image values with respect to the original was obtained.

We claim:

55 1. An electrophotographic process for producing selectively positive or negative copies of a given original comprising the steps of: uniformly corona charging a bi-chargeable photoconductive recording material comprising a photoconductive recording layer comprising an electrically insulating binder and dispersed therein a mixture of photoconductive zinc oxide particles and positively chargeable particles of the group consisting of barium sulphate, silica, and polyethylene, the ratio by weight in said layer of the photoconductive zinc oxide particles with respect to said positively chargeable particles ranging from 10:90 to less than 60:50, the recording layer containing the dispersed mixture of particles in a proportion with respect to the

binder material of from 50 to 97% by weight, the zinc oxide particles having a grain size in the range of 0.1 to 15 micron and the positively chargeable particles a grain size in the range of  $10^{-2}$  to 50 microns,

said uniform charge having one polarity for positive 5 copy and the opposite polarity for a negative copy, exposing said layer to a light image of said original to dissipate said charges in the exposed areas while

leaving the charges retained in the non-image areas, and developing the exposed sheets by contacting the same with toner particles charged with the same polarity for both positive and negative copies.

2. An electrophotographic process according to claim 1 wherein said original is a microfilm image.

\* \* \* \* \*